

1

2,955,900

## NEW COLOURING PROCESS

Timothy Leslie Dawson, Manchester, England, assignor to Imperial Chemical Industries Limited, London, England, a corporation of Great Britain

No Drawing. Filed Jan. 10, 1957, Ser. No. 633,387

10 Claims. (Cl. 8—31)

This invention relates to a new colouring process, and more particularly it relates to a new colouring process suitable for the application of basic dyestuffs and dyestuffs containing ternary or quaternary salt groups.

These latter dyestuffs may be applied to textile materials by conventional dyeing methods and then rendered insoluble by treatment of the dyed textile material with alkali to give dyeings having good light- and wash-fastness. When applied in this way the affinities of the dyestuffs for cellulosic materials are not entirely satisfactory and deep shades are not readily obtainable. It is known that deep shades are readily obtainable on cellulosic materials by impregnating with the dye-liquor and then drying before treating with alkali, but this method suffers from the defect that the dyestuff shows a tendency to migrate while the textile material is being dried and the final dyeings are uneven.

It has now been found that the affinity of cellulosic textiles, and more particularly of cotton and cuprammonium rayon textile materials for the above dyestuffs may be greatly increased by impregnating the said textile materials with a mixture of polyacrylic acid and an alkali metal salt of polyacrylic acid.

According to the invention, therefore, there is provided a process for colouring cellulosic textile material which comprises impregnating the said material with a mixture of a polymer of acrylic acid and one or more alkali metal or ammonium salts of a polymer of acrylic acid, thereafter dyeing the said material with a basic dyestuff or a dyestuff containing ternary or quaternary salt groups, and finally treating the dyed material with alkali to complete the fixation of the dyestuff.

As examples of cellulosic textile materials which may be coloured by the process of the invention there may be mentioned cotton, linen, cuprammonium rayon, and viscose rayon.

As examples of alkali-metal salts of polymers of acrylic acid which may be used in the process of the invention there may be mentioned sodium and potassium salts of polymers of acrylic acid.

The impregnation of the said textile material may be conveniently carried out by passing it through an aqueous solution containing both a polymer of acrylic acid and alkali or ammonium salt of the polymer and then drying. The solution may conveniently be obtained either by partial neutralisation of a polymer of acrylic acid with ammonia or a suitable alkali-metal hydroxide, carbonate or bicarbonate, or by partial acidification of a solution of an alkali-metal or ammonium salt of a polymer of acrylic acid. The polymer of acrylic acid (or alkali-metal or ammonium salt thereof) used may be obtained by any method known from the literature or used in practice for the manufacture of polymers of acrylic acid, for example by polymerisation of acrylic acid either catalytically or by heat, by polymerisation of acrylonitrile followed by either acid or alkaline hydrolysis and by polymerisation of esters of acrylic acid, for example ethyl acrylate, followed by hydrolysis of the polymer formed,

2

and such hydrolyses may be carried out on polymers either in the solid state or in an emulsified state. The products so obtained are substantially polymers of acrylic acid (or salts thereof) but may contain minor amounts of nitrile, amide or ester groups, depending on the method of preparation. Similar polymers may be obtained, if desired, by the co-polymerisation of mixtures of acrylic acid with minor amounts of co-polymerisable substances containing amide, nitrile or ester groups.

10 The total amount of the polymer of acrylic acid and salt thereof present in the solution may lie between 0.1 parts and 2.5 parts in each 100 parts by weight of the solution, but it is preferred to use a solution containing 0.2 to 0.5 parts in each 100 parts by weight of the solution.

15 Polymers of acrylic acid may be used which form solutions in 2 N sodium hydroxide having viscosities at 20° C. of not less than 2 centipoises and not more than 10 centipoises when 10 grams of the polymer are dissolved in sufficient 2 N aqueous sodium hydroxide to give a volume of 1 litre. It is preferable, however, to use a polymer of acrylic acid which gives such a solution in 2 N sodium hydroxide having a viscosity of not less than 2 and not more than 4 centipoises at 20° C.

20 25 The proportion of polymer of acrylic acid and salt thereof present in the solution used for impregnation of the textile materials may be such that the pH of the solution is not less than 3 and not more than 10, but it is preferred to use a proportion such that the pH of the 30 solution is not less than 5.5 and not more than 6.5

25 Suitable dyestuffs for use in the invention are for example those obtained by reacting chloromethyl derivatives of phthalocyanines with tertiary amines or thioureas as described in United Kingdom specification No. 587,636

30 35 and also dyestuffs obtained in a similar manner from chloromethyl derivatives of anthraquinone vat dyestuffs, for example dibenzanthrone and isodibenzanthrone, and from chloromethyl derivatives of azo pigments, for example 4:4' - di(6'-methylbenzthiazyl-)azobenzene. As 40 examples of basic dyestuffs which may be used, there may be mentioned Methylene Blue 2BS (Colour Index No. 922), Victoria Blue BS (Colour Index No. 729), Magenta PNS (Colour Index No. 677) and Auramine OS (Colour Index No. 655).

45 50 It has been found that the coloured textile materials obtained by the new process are considerably more resistant to removal of dyestuff by wet or dry abrasive treatments than are coloured textile materials obtained when the pretreatment with polyacrylic acid and polyacrylate is omitted.

55 When a bath-dyeing technique is used, that is the material is dyed on a winch or jig, the dye-liquor exhausts to a higher degree, and deeper shades are obtained than can be obtained on textile materials which have not been treated with polyacrylic acid and polyacrylate.

60 When a pad-dry or pad-steam dyeing technique is used, the pretreated textile material gives dyeings having a better colour value. When a pad-dry technique is used, dyestuff applied to pretreated textile materials shows much less tendency to migrate under adverse drying conditions.

The invention is illustrated but not limited by the following examples in which the parts are by weight.

### Example 1

65 A solution is prepared by dissolving 0.5 parts of a polymer of acrylic acid in 99.5 parts of water containing sufficient sodium hydroxide for the solution to have a pH of 5.7. Cotton limbric is passed through this solution and squeezed so as to give an increase in weight of 100% over the weight of the cloth which is then dried at 100° C.

100 parts of the pre-treated cotton limbric are thoroughly rinsed in water, then introduced into 5000 parts of dye-liquor containing 1.5 parts of the dyestuff obtained by reacting copper tri-(chloromethyl)-phthalocyanine with tetramethylthiourea. The dyebath is heated to the boiling point during 30 minutes, and maintained at this temperature for 30 minutes, with continual agitation of the fabric. During this time, the pH of the dye-bath is maintained at 3.5 by the addition of acetic acid.

The cotton limbric is then removed, rinsed in water and immersed for 5 minutes in a boiling solution containing 20 parts of sodium carbonate in 1000 parts of water. It is then boiled for 10 minutes in a solution containing 1 part of a detergent obtained by condensing ethylene oxide with an alkyl phenol in 1000 parts of water, then rinsed with water and dried.

The uptake of dyestuff on the cotton limbric when measured by spectrophotometric examination of the exhaust liquor is found to be 1.25 parts. 100 parts of cotton limbric which had not been pretreated when dyed similarly give an uptake of 0.6 parts of dyestuff.

The polymer of acrylic acid used in this example is obtained by catalytic polymerisation of acrylic acid and forms a solution in 2 N sodium hydroxide having a viscosity of 2.4 centipoises at 20° C. when 10 parts of polyacrylic acid are dissolved in sufficient 2 N sodium hydroxide to give a total volume of 1 litre.

#### Example 2

100 parts of cuprammonium rayon sateen pretreated and dyed as described for the cotton limbric in Example 1. The dyestuff uptake is 1.48 parts. Cuprammonium rayon sateen which is not pretreated has a dyestuff uptake of 0.6 parts.

#### Example 3

The solution of polymer of acrylic acid used in Example 1 to impregnate the cotton limbric is replaced by a solution of 1 part of polymer of acrylic acid in 99 parts of water, containing sufficient sodium hydroxide to have a pH of 5.7, and the amount of dyestuff in the dyebath is increased to 2.5 parts. A dye uptake of 2.2 parts is obtained.

#### Example 4

Cotton limbric is pretreated as described in Example 1. The fabric is then passed through a solution containing 10 parts of the dyestuff described in Example 1 and 5 parts of acetic acid in 1000 parts of water and squeezed so as to give an increase in weight of 80% over the weight of the cloth, which is then dried at 100° C., and passed through a boiling solution containing 5 parts of sodium carbonate in 1000 parts of water. It is then treated with detergent, rinsed and dried as described in Example 1.

When cotton limbric which has not been pre-treated is dyed and fixed in the same way, more of the dyestuff is removed from the dyeing during the treatment with sodium carbonate solution than is removed from the pre-treated cotton limbric and more is removed from the dyeing which has not been pre-treated when exposed to friction under wet or dry conditions than is removed from the pre-treated cotton limbric.

#### Example 5

Both pre-treated and non-pretreated strips of cotton limbric are passed through a solution containing 10 parts of the dyestuff described in Example 1 and 5 parts of glacial acetic acid in 1000 parts of water.

The strips are then separately wound several times round a cylinder and dried in a stream of warm air. The dyestuff on the strips of cotton limbric which have been pretreated show much less tendency to migrate to the outer layers of the cotton limbric than does the dyestuff on the untreated strips.

#### Example 6

100 parts of cotton limbric are pretreated as in Example 1 and dyed, fixed and dried as described therein but using only sufficient dyestuff in the dyebath to give an uptake of 0.5 parts of dyestuff. 100 parts of cotton limbric which has not been pretreated are also dyed, fixed and dried to give an uptake of 0.5 part of dyestuff.

The pretreated cotton limbric has much greater resistance to removal of the dyestuff under dry and wet conditions than the cotton limbric which has not been pretreated.

#### Example 7

A mixture of 486 parts of water and 5 parts of a 5% aqueous solution of sulphuric acid is heated to 40° C. and 2 parts of ammonium persulphate in 8 parts of water, 2 parts of sodium meta-bisulphite in 8 parts of water and 60 parts of acrylonitrile are added. Immediate polymerisation occurs and the temperature of the mixture rises to 68° C. The temperature is adjusted to 60° C. and the mixture is maintained at this temperature for one hour. 46 parts of sodium hydroxide are added to the polymer slurry and the mixture is heated at 90-95° C. for 24 hours, the volume of the solution being kept constant during this time by the addition of water. Analytical estimation of the product indicates that the polyacrylonitrile is 85 parts hydrolysed to sodium polyacrylate. The polymer forms a solution having a viscosity of 3.5 centipoises at 20° C. when a quantity equivalent to 10 parts of polyacrylic acid is dissolved in sufficient 2 N sodium hydroxide to give a total volume of one litre.

The above polymer solution is diluted to give a solution equivalent to 0.5 part of polyacrylic acid in 99.5 parts of water containing sufficient acetic acid for the solution to have a pH of 5.7. Cotton limbric is passed through this solution and squeezed so as to give an increase in weight of 100% over the weight of the cloth which is then dried at 100° C.

100 parts of the pretreated cotton limbric is rinsed in water and then introduced into 5,000 parts of dye liquor containing 1.5 parts of the dyestuff obtained by reacting copper tri(chloromethyl)phthalocyanine with tetramethylthiourea. The dyebath is heated to the boiling point during 30 minutes and maintained at this temperature for 30 minutes with continual agitation of the fabric. During this time the pH of the dyebath is maintained at 3.5 by the addition of acetic acid. The cotton limbric is then removed, rinsed in water and immersed for 5 minutes in a boiling solution containing 20 parts of sodium carbonate in 1000 parts of water. It is then boiled for 10 minutes in a solution containing 1 part of a detergent obtained by condensing ethylene oxide with alkyl phenol in 1000 parts of water, rinsed with water and dried. The uptake of dyestuff on the cotton limbric when measured by spectrophotometric examination of the exhaust liquor is found to be 1.26 parts per 100 parts of cotton limbric. Cotton limbric which has not been pretreated when dyed similarly gives an uptake of 0.6 part of dyestuff per 100 parts of cotton limbric.

#### Example 8

A mixture of 500 parts of water, 3.8 parts of sodium carbonate and 8 parts of Turkey Red Oil is heated to 90° C. and stirred vigorously while simultaneously from separate vessels there are added during 1½ hours 400 parts of ethyl acrylate monomer, 8 parts of Turkey Red Oil in 200 parts of water, and 1.32 parts of ammonium persulfate in 100 parts of water. Care is taken to maintain the rates of addition of monomer, catalyst and surface active agent constant. When the additions are complete, the temperature of the dispersion is maintained at 90-92° C. for a further hour to complete the polymerization.

56 parts of sodium hydroxide are dissolved in 100

parts of water and this solution is added to 500 parts of an aqueous dispersion of polyethyl acrylate prepared as described above. The mixture is stirred and heated to about 90° C. and maintained at 80-90° for 3 hours. Titration of the residual sodium hydroxide with standard acid solution indicates that the polyethyl acrylate is 75% hydrolysed to sodium polyacrylate. The polymer obtained forms a solution having a viscosity of 8.25 centipoises at 20° C. when a quantity equivalent to 10 parts of polyacrylic acid is dissolved in sufficient 2 N sodium hydroxide to give a total volume of one litre.

The above polymer solution is diluted to give a solution equivalent to 0.5 part of polyacrylic acid in 99.5 parts of water containing sufficient acetic acid for the solution to have a pH of 5.7. 100 parts of cotton limbric is pretreated and dyed as described in Example 7 using the above solution for the pretreatment. The uptake of dyestuff is 1.09 part per 100 parts of cotton limbric.

*Example 9*

A mixture of 350 parts of water, 2.5 parts of sodium hydroxide and 10 parts of Turkey Red Oil is heated to 90° C. and to this mixture are added 750 parts of ethyl acrylate monomer, 100 parts of Turkey Red Oil in 200 parts of water and 6.25 parts of ammonium persulphate in 200 parts of water. Polymerisation is effected as described in Example 8. 45.2 parts of sodium hydroxide are dissolved in 500 parts of water and this solution is added to 200 parts of the aqueous dispersion of polyethyl acrylate prepared as described above. Hydrolysis is carried out as described in Example 8 except that the total time of hydrolysis is 16 hours. Titration of the residual sodium hydroxide with standard acid solution indicates that the polyethyl acrylate is 95% hydrolyzed to sodium polyacrylate. The polymer obtained forms a solution having a viscosity of 2.04 centipoises at 20° C. when a quantity equivalent to 10 parts of polyacrylic acid is dissolved in sufficient 2 N sodium hydroxide to give a total volume of one litre. The above polymer solution is diluted to give a solution equivalent to 0.5 part of polyacrylic acid in 99.5 parts of water containing sufficient acetic acid for the solution to have a pH of 5.7. 100 parts of cotton limbric is pretreated and dyed as described in Example 7 using the above solution for the pretreatment. The uptake of dyestuff is 1.23 parts per 100 parts of cotton limbric.

*Example 10*

A solution containing 80 parts of acrylic acid monomer in 20 parts of water is refluxed at about 140° C. After 10 minutes polyacrylic acid begins to separate from the monomer solution. After heating for a further 45 minutes the solid polymer is separated from the residual solution and dried giving 75 parts of polyacrylic acid. The polymer forms a solution in 2 N sodium hydroxide having a viscosity of 2.0 centipoises at 20° C. when 10 parts are dissolved in sufficient 2 N sodium hydroxide to give a total volume of one litre.

A solution of this product is prepared by dissolving 0.5 part in 99.5 parts of water containing sufficient sodium hydroxide for the solution to have a pH of 5.7. 100 parts of cotton limbric is pretreated and dyed as described in Example 7 using the above solution for the pretreatment. The dyestuff uptake is 1.03 part per 100 parts of cotton limbric.

Similar results are obtained if the polymer solution is adjusted to pH 5.7 with either ammonium or potassium hydroxide in place of sodium hydroxide.

*Example 11*

100 parts of cotton limbric is pretreated and dyed as described in Example 7 except that the dyestuff is replaced by the dye obtained by reacting chloromethyl-4:4'-di(6"-methylbenzthiazyl)azobenzene with tetramethylthiourea. The dyestuff uptake is 1.25 parts per 100 parts of cotton limbric. 100 parts of cotton limbric which has not been

pretreated when dyed similarly gives an uptake of 0.6 parts of dyestuff.

*Example 12*

5 100 parts of cotton limbric is pretreated and dyed as described in Example 7 except that the dyestuff is admixed with an equal weight of the dyestuff used in Example 11. The uptake of the green dyestuff mixture is 1.31 parts per 100 parts of cotton limbric. 100 parts of cotton limbric which has not been pretreated when dyed similarly gives an uptake of 0.6 parts of dyestuff.

*Example 13*

15 100 parts of cuprammonium rayon sateen is pretreated and dyed as described for the cotton limbric in Example 7. The dyestuff uptake is 1.48 parts. Cuprammonium rayon sateen which is not pretreated has a dyestuff uptake of 0.6 part per 100 parts of cuprammonium rayon sateen.

*Example 14*

20 100 parts of cotton limbric is pretreated and dyed as described in Example 7 except that the concentration of the polymer solution is increased until equivalent to 1 part of polyacrylic acid in 99 parts of water containing sufficient acetic acid for the solution to have a pH of 5.7. The amount of dyestuff in the dyebath is increased to 2.5 parts. A dye uptake of 2.2 parts per 100 parts of cotton limbric is obtained.

*Example 15*

25 30 35 Cotton limbric is pretreated as described in Example 7. The fabric is then passed through a solution containing 10 parts of the dyestuff described in Example 7 and 5 parts of acetic acid in 1,000 parts of water and squeezed so as to give an increase in weight of 80% over the weight of the cloth, which is then dried at 100° C. and passed through a boiling solution of sodium carbonate in 100 parts of water. It is then treated with detergent as described in Example 7.

40 45 When cotton limbric which has not been pretreated is dyed and fixed in the same way, more of the dyestuff is removed from the dyeing during the treatment with sodium carbonate solution than is removed from the pretreated cotton limbric, and more is removed from the dyeing which has not been pretreated when exposed to friction under wet or dry conditions than is removed from the pretreated cotton limbric.

*Example 16*

50 55 Both pretreated and non-pretreated strips of cotton limbric are passed through a solution containing 10 parts of the dyestuff described in Example 7 and 5 parts of glacial acetic acid in 1000 parts of water. The strips are then separately wound several times round a cylinder and dried in a stream of warm air. The dyestuff of the strips of cotton limbric which have been pretreated show much less tendency to migrate to the outer layers of the cotton limbric than does the dyestuff on the untreated strips.

*Example 17*

60 65 70 100 parts of cotton limbric is pretreated as described in Example 7 and dyed, fixed and dried as described therein but using only sufficient dyestuff in the dyebath to give an uptake of 0.5 part of dyestuff. 100 parts of cotton limbric which have not been pretreated is also dyed, fixed and dried to give an uptake of 0.5 part of dyestuff. The pretreated cotton limbric has much greater resistance to removal of the dyestuff by abrasion under dry and wet conditions than the cotton limbric which has not been pretreated.

*Example 18*

100 parts of cotton limbric is pretreated as described in Example 7. The fabric is then introduced into 5000 parts of dye liquor containing 0.5 part of Victoria Blue

BS (Colour Index No. 729) and 2.5 parts of glacial acetic acid. The dyebath is heated to 70° C. during 30 minutes and maintained at this temperature for 30 minutes, with continual agitation of the fabric.

The cotton limbric is then removed, rinsed well in water and dried. The uptake of dyestuff on the cotton limbric when measured by spectrophotometric examination of the exhaust liquor is found to be 0.4 parts per 100 parts of cotton limbric. 100 parts of cotton limbric which has not been pretreated similarly gives an uptake of 0.21 parts of dyestuff.

*Example 19*

100 parts of cotton limbric is pretreated as described in Example 7. The fabric is then introduced into 5,000 parts of dye liquor containing 0.5 part of Methylene Blue 2BS (Colour Index No. 922) and 2.5 parts of glacial acetic acid. The dyebath is heated to 70° C. during 30 minutes and maintained at this temperature for 30 minutes with continual agitation of the fabric. The cotton limbric is then removed, rinsed well in water and dried. The uptake of dyestuff on the cotton limbric is found to be 0.36 part per 100 parts of cotton limbric. 100 parts of cotton limbric which has not been pretreated when dyed similarly gives an uptake of 0.1 part of dyestuff.

What I claim is:

1. Process for colouring cellulose textile material which comprises impregnating the said material with an aqueous solution of a mixture of a polymer of acrylic acid and at least one salt of the group consisting of alkali metal and ammonium salts of a polymer of acrylic acid, thereafter dyeing the material with a dyestuff selected from the class consisting of dyestuffs containing ternary salt groups and dyestuffs containing quaternary salt groups, which are rendered insoluble in water by alkali, and finally treating the dyed material with alkali to complete the fixation of the dyestuff.

2. Process for colouring cellulose textile material as claimed in claim 1 wherein the alkali-metal salts of polymers of acrylic acid are selected from the group consisting of the sodium and potassium salts.

3. Process for colouring cellulose textile material as claimed in claim 1 wherein said polymer of acrylic acid is one which forms a solution in 2 N sodium hydroxide having a viscosity at 20° C. of not less than 2 centipoises and not more than 10 centipoises, when 10 grams of the

polymer are dissolved in sufficient 2 N aqueous sodium hydroxide to give a volume of 1 litre.

4. Process for colouring cellulose textile material as claimed in claim 1 wherein the proportion of polymer of acrylic acid and salt thereof present in the solution used for impregnation of the textile materials is such that the pH of the solution is not less than 3 and not more than 10.

5. Process for colouring cellulose textile material as claimed in claim 1 wherein said polymer of acrylic acid is one which forms a solution in 2 N sodium hydroxide having a viscosity at 20° C., of not less than 2 centipoises and not more than 4 centipoises when 10 grams of the polymer are dissolved in sufficient 2 N aqueous sodium hydroxide to give a volume of 1 litre.

10 6. Process for colouring cellulose textile material as claimed in claim 1 wherein the proportion of polymer of acrylic acid and salt thereof present in the solution used for impregnation of the textile materials is such that the pH of the solution is less than 5.5 and not more than 6.5.

7. Process for colouring cellulose textile material as claimed in claim 1 wherein the impregnation of the said textile material is carried out by passing it through an aqueous solution containing both said polymer of acrylic acid and salt thereof and then drying the impregnated material prior to the dyeing step.

8. Process for colouring cellulose textile material as claimed in claim 7 wherein the total amount of the polymer of acrylic acid and salt thereof present in the solution is between 0.1 part and 2.5 parts in each 100 parts by weight of the solution.

9. Process for colouring cellulose textile material as claimed in claim 7 wherein the total amount of the polymer of acrylic acid and salt thereof present in the solution is between 0.2 to 0.5 part by weight of the solution.

10. Cellulose textile materials whenever coloured by a process as defined in claim 1.

References Cited in the file of this patent

UNITED STATES PATENTS

|           |         |                |
|-----------|---------|----------------|
| 2,215,196 | Schlack | Sept. 17, 1940 |
| 2,343,095 | Smith   | Feb. 29, 1944  |
| 2,764,570 | Kowolik | Sept. 25, 1956 |

FOREIGN PATENTS

|         |               |              |
|---------|---------------|--------------|
| 433,210 | Great Britain | Aug. 9, 1935 |
|---------|---------------|--------------|